# EUROPEAN PATENT SPECIFICATION

(11) **EP 0 125 144 B1**
(45) Date of publication and mention of the grant of the patent: **11.10.1989**
(21) Application number: 84303141.0
(22) Date of filing: 09.05.1984
(51) Int. Cl.: C10M 137/04, C07F 9/141

(54) **Functional fluids and lubricants having improved water tolerance**
Funktionelle Flüssigkeiten und Schmiermitteln mit verbesserter Wassertoleranz
Fluides fonctionnels et lubrifiants ayant une tolérance à l'eau ameliorée

(30) Priority: 10.05.1983 US 493398
(43) Date of publication of application: 14.11.1984
(73) Proprietor: EXXON RESEARCH AND ENGINEERING COMPANY, Florham Park, New Jersey 07932-0390 (US); Argus Chemical Corporation, Brooklyn New York 11231 (US)
(72) Inventor: Brecker, Lawrence Robert, Brooklyn New York (US); Loeffler, Otto Ernest, Woodbridge New Jersey (US); Abramoff, Charles, New York, NY (US); Cleveland, Wiliam, Kennth, Roselle New Jersey (US); Wosatka, Susan Jean, Linden New Jersey (US)
(74) Representative: Bawden, Peter Charles

(56) References cited:
- US-A- 2 241 244
- US-A- 4 346 148

## Description

This invention relates to functional fluids and lubricants which exhibit improved water tolerance properties. More particularly, the invention relates to mineral oil or synthetic oil based functional fluid compositions which contain effective amounts of certain oil-soluble, alkoxypolyethyleneoxy mono- or diacid phosphite ester additives, which additives are highly effective in improving the water tolerance properties of such compositions.

U.S. Patent No. 2,280,450 describes hydrocarbon oils of improved resistance to corrosion containing a small amount of a substantially stable oil-soluble water-in-soluble reaction product of tricresyl phosphite and octyl phenoxyethanol. The mole ratio of tricresyl phosphite to octyl phenoxyethanol varies from 1:1 to about 1:2.5. The reaction product is described as a complex ester of phosphorous acid, which may or may not contain unreacted octyl phenoxyethanol. The product is not however an acid phosphite, and it is not suggested that the water tolerance of the resulting composition is improved.

U.S. Patent No. 3,583,915 provides industrial fluid compositions and lubricant compositions containing improved load-carrying additives, including diorgano hydrogen phosphonate in which at least one organic group is an aliphatic group containing at least fourteen carbon atoms in admixture with an active sulfur compound.

U.S. Patent No. 3,652,410 provides multifunctional lubricant additive compositions and lubricating oils containing, among other things, an organic acid phosphate or organic phosphite containing at least one alkyl or alkenyl group having from about 12 to about 24 carbon atoms. Also present is a mineral oil soluble or dispersible basic detergent, a mineral oil antioxidant, a sulfurized fat, or an alkyl sulfide or alkyl polysulfide.

U.S. Patent No. 4,346,148 and U.S. Patent No. 4,358,509 describe reaction products of alkoxylated alkyl phenol and a phosphorus trihalide which are included in lubricating compositions useful in metal-working operations, imparting corrosion resistance, extreme pressure properties, and protection against wear of working parts.

U.S. Patent No. 3,115,465 provides antioxidant combinations for organic materials, including lubricants, comprising an oil-soluble phosphite ester having the formula: wherein R₁ and R₂ are alkyl, alkoxyalkyl, haloalkyl, cycloalkyl, halocycloaikyl, aralkyl, aryl, alkaryl, haloaryl, or haloalkaryl radicals and R₃ is hydrogen or one of the aforesaid radicals; and from about 0.01 to about 5, preferably 0.25 to 2%, by weight based on the oil of a methylene bis-phenol having the formula: wherein R₄ is an alkyl group containing 3 to 12 carbon atoms, the group being branched on its alpha carbon atom, and Rₛ is an alkyl group of 1 to 12 carbon atoms. United States Patent 2241244 discloses lubricants containing certain similar phosphite esters with alkyl groups of 8 or fewer carbon atoms.

None of the foregoing references disclose the improvement in water tolerance properties achieved in accordance with the present invention. Water compatability is a highly significant property of functional fluids and lubricants, which, under severe conditions, come into contact with water and in the absence of acceptable water tolerance properties the fluid will have its lubricating and power transmission properties substantially reduced. The specifications of many equipment manufacturers require that fluids and lubricants used therein have certain water tolerance properties, for example, fluids for use in agricultural machinery, such as tractor fluids.

In accordance with the present invention, there have been discovered improved function fluids and lubricating compositions comprising major amount of a synthetic or mineral oil or lubricating viscosity and an amount, effective to improve the water tolerance properties of the composition, of an oil-soluble alkoxypolyethyleneoxy acid phosphite ester additive of the formula: wherein R₁ is alkyl or alkenyl containing 9 or more carbon atoms and R₂ is OH, alkoxy, oxy-alkenyl, or R₁O[CH₂CH₂O]ₓ; in which the total number of carbon atoms in the alkyl, alkenyl, alkoxy or oxyalkenyl groups is 9 to 36; and x is a number (which can be a whole number or a fractional number) representing the average number of [CH₂CH₂0] groups and ranges from 2 to 4. Preferred phosphite additives are those wherein x is 2, 2.5, 3.5 or 4.

In R₂ the alkyl and alkenyl groups include octyl, 2-ethylhexyl, isooctyl, tertiary-octyl and octenyl and in R, and R₂ they include onyl, isononyl, tertiary-nonyl, secondary nonyl, decyl, isodecyl, undecyl, doecyl, tridecyl, palmityl (i.e., hexadecyl), stearyl, (i.e., octadecyl), and isostearyl (i.e., isooctadecyl); octenyl, nonenyl, decenyl, dodecenyl, oleyl (i.e., octadecenyl), linoleyl (i.e., octadecadineyl) and linolenyl (i.e., octadecatrienyl).

Acid phosphites according to the invention include di(nonyl-di(ethyleneoxy)) phosphite, di(isodecyl- tri(ethyleneoxy)) phosphite, di(hexadecyl-tetra-(ethyleneoxy)) phosphite, di(octadecyl-tri(ethyleneoxy)) phosphite, octadecyl-di(ethyleneoxy)phosphite, nonyl-di(ethyleneoxy) nonyl phosphite, isodecyl- tri(ethyleneoxy) octadecatrienyl phosphite, hexadecyl-tetra(ethyleneoxy) octadecyl phosphite, octadecyl- tri(ethyleneoxy) octadecyl phosphite, and octadecyl di(ethyleneoxy) octadecyl phosphite.

The oil-soluble phosphite ester additive of this invention will provide effective water tolerance properties to a wide variety of functional fluid and lubricating compositions and these include hydraulic fluids, compressor oils, pumps oils, tractor fluids and universal tractor fluid compositions, gear oils, hydrostatic transmission oils, power shift transmission fluids and the like. Such functional fluids and lubricating compositions will also contain a number of conventional additives in amounts as required to provide their normal attendant functions. Such additives include viscosity modifiers or viscosity index improvers, corrosion inhibitors, oxidation inhibitors, friction modifiers, dispersants, demulsifiers, anti-foam agent, anti-wear agents, pour point depressants, seal swellants and other special purpose additives.

Typical viscosity modifiers include polyisobutylene, ethylene-propylene copolymers, polymethacrylates, styrene-acrylic ester copolymers and vinyl monomer unsaturated dicarboxylic acid (or ester) copolymers. Corrosion inhibitors include zinc dialkyl dithiophosphates and phosphosulfurized hydrocarbons and reaction products thereof with alkaline earth metal oxides or hydroxides, preferably in the presence of alkyl phenols and alkyl phenol thioethers. Oxidation inhibitors are illustrated by alkaline earth metal salts of alkyl (C₅―C₁₂) phenorthioethers.

Dispersants are well known in the art and include oil-soluble alkenyl succinimides, e.g., the reaction products of polyisobutenyl succinic anhydrides with ethylene amines and borated derivatives. Exemplary pour point depressents are C₈―C₁₈ dialkylfumarate/vinyl acetate copolymers, polymethacrylates and wax- . naphthalene condensation products. Anti-foam agents are typically polysiloxane materials such as silicone oil and polydimethyl siloxane; anti-wear agents include zinc dialkyl (or diaryl) dithio-phosphates and magnesium sulfonates. Seal swellants are typified by mineral oils that provoke swelling, Cₛ-C,₃ aliphatic alcohols and C₁₀―C₆₀ hydrocarbon esters having 2-4 ester linkages such as dihexylphthalate.

The oil-soluble phosphite ester additive of this invention will be present in amounts effective to provide acceptable water tolerance properties to the particular composition and the desired amount will vary according to the service conditions but generally the additives of this invention will be present in an amount of about 0.05 to 5% by weight, based on the weight of the total lubricating oil or functional fluid composition and preferably from about 0.2 to 2% by weight percent.

Typical base oils for such functional fluids and lubricating compositions include a wide variety of hydrocarbon mineral oils such as naphthene base, paraffin base, and mixtures thereof having a lubricating viscosity range of about 34 to 45 Saybolt Universal Seconds (SUS) at 35°C. Examples of synthetic oils useful in the composition of the present invention include olefin oligomers, alkylated aromatics, polybutene oils, cycloaliphatic compounds, dibasic acid esters, polyol esters, polyglycerol fluids, phosphate esters, silicone oils and halogenated hydrocarbon fluids and mixtures thereof.

The following examples illustrate the preferred embodiments of the oil soluble phosphite ester additives of this invention: (EO refers to ethylene oxide).

### Example I

### Di(C₉―C₁₁ alkyl 2.5 EO) phosphite

159.8 g of triphenyl phosphite (97%) and 405 g of (mixed alkyl(oxyethylene)₂.₅ alcohols, the alkyl having from nine to eleven carbon atoms, and 0.6 g of K_{Z}C0₃ were heated at 85°C for three hours. Vacuum was then applied (6 mm) with heating to a maximum temperature of 170°C to remove phenol. The weight of volatiles collected was 150.9 g (theory 145.8). To the transesterified product 15.63 g of phosphorous acid was added the agitation and the mixture heated to 85°C for 5 hours with agitation, giving clear reaction product having the formula:

### Example II

Di(C₁₂―C₁₅ alkyl-3EO) phosphite was prepared from triphenyl phosphite (97%), and (mixed alkyl)oxyethylene)₃ alcohols, the alkyl having from eleven to fifteen carbon atoms) using the procedure of Example I. The compound has the formula:

### Control A

Di(C₁₂―C₁₅ alkyl-7EO) phosphite was prepared from triphenyl phosphite (97%), and mixed C₁₂―C₁₅ (oxyethylene)₇ alcohols, using the procedure of Example I. The compound has the formula:

### Control B

Ethoxylated nonyl phenol (9.5EO) phosphite was prepared from triphenyl phosphite and ethoxylated nonylphenol using the procedure of Example I. The compound has the formula:

### Example III

Mono (C₉₋₁₁ alkyl 2.5EO) mono oleyl phosphite was prepared from triphenyl phosphite ((mixed alkyl oxyethylene)₂.ₛ alcohols, the alkyl having from nine to eleven carbon atoms), and oleyl alcohol using the procedure of Example I. The compound has the formula:

Typical functional fluids or lubricating composition of the present invention will contain a number of conventional additives in typical amounts as required to provide their normal attendant functions. Such additive components and their usual ranges are set forth below.

The foregoing composition is referred to as Base Fluid and a tractor hydraulic fluid corresponding to the Base Fluid was evaluated for water tolerance with various additives as set forth below. The mineral oil used in the Base Fluid had a kinematic viscosity of 69.8 centistokes (69.8 x 10⁻²m²S⁻¹ at 37.08°C and 14.5 centistokes (14.5 x 10⁻²m²S⁻¹ at _{98.9°C}.

The test used was the International Harvester Water Tolerance Test IH BI-7; January, 1980 contained in the International Harvester Engineering Materials Specification for Combination Hydraulic and Transmission Fluid.

The test is described as follows:

### Apparatus required

(1) Mechanical paint shaker, Red Devil No. 30 or equivalent.
(2) 118 ml bottle with cap.
(3) Graduated cylinder, 100 ml.
(4) 100 ml centrifuge tube according to ASTH Designation D 2273-67.
(5) Pipette or syringe capable of delivering 1.0 ml.
(6) Stopper to fit centrifuge tube.

### Procedure

(1) Add 1 ml distilled water to 99 ml hydrocarbon oil in the 118 ml bottle.
(2) Shake the prepared sample for 5 minutes in the mechanical shaker.
(3) Transfer immediately to the 100 ml centrifuge tube.
(4) Stopper and let the agitated solutions stand undisturbed in a vertical position for 168 hours (7 days at 70 to 80°F, 21 to 27°C), then examine for emulsion, water, clearness and sediment.

### Report

(1) Level of emulsion, water and sediment to the nearest 0.1 ml.
(2) The clearness or turbidity of the solution.

### Example IV

The results of evaluations are tabulated below in the Table, The data include comparisons with Control A, Control B and two commercially available Surfactants A (sorbitan oleate) and B (ethoxylated fatty acid ester of sorbitol anhydride). All additives were employed in the same Base Fluid at concentration of 1 % by weight.

## Claims

1. A functional fluid composition comprising a major amount of a synthetic or mineral oil of lubricating viscosity and 0.05 to 5 wt.% by weight of the oil of an oil soluble phosphite ester additive of the formula: wherein R₁ is alkyl or alkenyl containing 9 or more carbon atoms, and R₂ is OH, alkoxy, oxy-alkenyl or R,O (CH₂CH₂O)x, in which the total number of carbon atoms in the alkyl, alkenyl, alkoxy or oxyalkenyl groups is from 9 to 36, and x is a number representing the average number of (CH₂CH₂0) groups and is within the range from 2 to 4.

2. A composition according to claim 1 in which x is 2, 2.5, 3, 3.5 or 4.

3. A composition according to claim 1 or claim 2, in which R, is alkyl having from nine to eleven carbon atoms.

4. A composition according to claim 1 or claim 2, in which R, is alkyl having from twelve to fifteen carbon atoms.

5. A composition according to claim 1 in which the phosphite ester is

6. A composition according to claim 1 in which the phosphite ester is and the oil is a hydrocarbon mineral oil.

7. A composition according to claim 1 in which the phosphite ester is

8. A composition according to any of claims 1 to 7, for use as a tractor fluid.

9. A hydrocarbon oil composition according to any of claims 1 to 8, in which the amount of the additive is within the range of from 0.2 to 2% by weight of the oil.

10. The use to improve the water tolerance of a functional fluid composition comprising a major amount of a synthetic or mineral oil of lubricating viscosity and 0.05 to 5 wt.% by weight of the oil of an oil soluble.phosphite ester additive of the formula: wherein R, is alkyl or alkenyl containing 9 or more carbon atoms and R₂ is OH, alkoxy, oxy-alkenyl, or R₁O(CH₂CH₂O)ₓ, in which the total number of carbon atoms in the alkyl, alkenyl, alkoxy or oxyalkenyl groups is 9 to 36; and x is a number representing the average number of (CH₂CH₂0) groups and ranges from 2 to 4.

## Patentansprüche

1. Funktionsfluidzusammensetzung (Arbeitsfluidzusammensetzung). die eine überwiegende Menge eines synthetischen Öls oder eines Mineralöls mit Schmiermittelviskosität und 0,05 is 5 Gew.% bezogen auf das Öls eines öllöslichen Phosphitesteradditivs mit der Formel: enthält, in der R, ein 9 oder mehr Kohlenstoffatome enthaltender Alkyl- oder Alkenylrest is und R₂ eine OH-Gruppe, ein Alkoxyrest, ein Oxyalkenylrest oder R₁O (CH₂CH₂0)x is, wobei die Gesamtzahl der Kohlenstoffatome in den Alkyl-, Alkoxy- oder Oxyalkenylgruppen 9 bis 36 beträgt und x eine Zahl im Bereich von 2 bis 4 ist, die die durchschnittliche Zahl der (CH₂CH₂0)-Gruppen wiedergibt.

2. Zusammensetzung nach Anspruch 1, in der x, 2, 2,5, 3, 3,5 oder 4 ist.

3. Zusammensetzung nach Anspruch 1 oder 2, in der R₁ ein Alkylrest mit 9 bis 11 Kohlenstoffatomen ist.

4. Zusammensetzung nach Anspruch 1 oder 2, in der R₁ ein Alkylrest mit 12 bis 15 Kohlenstoffatomen ist.

5. Zusammensetzung nach Anspruch 1, in der der Phosphitester ist.

6. Zusammensetzung nach Anspruch 1, in der der Phosphitester ist und das Öl ein Kohlenwasserstoffmineralöl ist.

7. Zusammensetzung nach Anspruch 1, in der der Phosphitester ist.

8. Zusammensetzung nach einem der Ansprüch 1 bis 7 zur Verwendung als Traktorfluid.

9. Kohlenwaserstoffölzusammensetung nach einem der Ansprüche 1 bis 8, in der die Additivmenge im Bereich von 0,2 bis 2 Gew.% bezogen aud das Öl beträgt.

10. Verwendung zur Verbesserung der Wassertoleranz einer Funktionsfluidzusammensetzung, die eine überwiegende Menge enthält, in der R, ein 9 oder mehr Kohlenstoffatome enthaltender Alkyl- oder Alkenylrest is und R₂ eine OH-Gruppe, ein Alkoxyrest, ein Oxyalkenylrest oder R₁O (CH₂CH₂0)x is, wobei die Gesamtzahl der Kohlenstoffatome in den Alkyl-, Alkoxy- oder Oxyalkenylgruppen 9 bis 36 beträgt und x eine Zahl im Bereich von 2 bis 4 ist, die die durchschnittliche Zahl der (CH₂CH₂0)-Gruppen wiedergibt.

## Revendications

1. Composition de fluide fonctionnel, comprenant une quantité dominante d'une huile synthétique ou minerale der viscosité propre à la lubrication et 0,05 à 5% en poids, par rapport au poids d'huile, d'une additif qui est un ester phosphitique soluble dans l'huile, répondant à la formule: dans laquelle R, est un groupe alkyle ou alcènyle contenant 9 ou plus de 9 atomes de carbone et R₂ est un groupe OH, alkoxy, oxy-alcényle ou R₁O (CH₂CH₂0)x, où le nombre total d'atomes de carbone dans les groupes alkyle, alcényle alkoxy ou oxyalcényle est de 9 à 36 et x est un nombre représentant le nombre moyen de groupes (CH₂CH₂0) et se situe dans l'intervalle de 2 à 4.

2. Composition suivant la revendication 1, dans laquelle x est égal 2, 2,5, 3, 3,5 ou 4.

3. Composition suivant la revendication 1 ou la revendication 2, dans lauelle R₁ est un groupe alkyle ayant neuf à onze atomes de carbone.

4. Composition suivant la revendication 1 ou la revendication 2, dans lauelle R₁ est un groupe alkyle ayant douze à quinze atomes de carbone.

5. Composition suivant la revendication 1, dans laquelle l'ester phosphitique répond à la formule:

6. Composition suivant la revendication 1, dans laquelle l'ester phosphitique répond à la formule: et l'huile est une huile minérale hydrocarbonée.

7. Composition suivant la revendication 1, dans laquelle l'ester phosphitique répond à la formule:

8. Composition suivant l'une quelconque des revendications 1 à 7, destinée à être utilisée comme fluide pour tracteur.

9. Composition d'huile hydrocarbonée suivant l'une quelconque des revidications 1 à 8, dans laquelle la quantité d'additif se situe dans l'intervalle de 0,2 à 2% en poids de l'huile.

10. Utilisation pour améliorer la tolérance à l'eau d'une composition de fluide fonctionnel comprenant une quantité dominante d'une huile synthétique ou minérale de viscosité propre à la lubrication et 0,05 à 5% en poids, par rapport au poids de l'huile, d'un additif qui est un ester phosphitique soluble dans l'huile de formule dans laquelle R₁ est un groupe alkyle ou alcènyle contenant 9 ou plus de 9 atomes de carbone et R₂ est un groupe OH, alkoxy, oxy-alcényle ou R₁0 (CH₂CH₂0)x, où le nombre total d'atomes de carbone dans les groupes alkyle, alcényle alkoxy ou oxyalcényle est de 9 à 36 et x est un nombre représentant le nombre moyen de groupes (CH₂CH₂0) et se situe dans l'intervalle de 2 à 4.
